# EUROPEAN PATENT SPECIFICATION

(11) **EP 3 642 382 B1**
(45) Date of publication and mention of the grant of the patent: **31.03.2021**
(21) Application number: 18729895.5
(22) Date of filing: 28.05.2018
(51) Int. Cl.: C23C 10/60, C23C 10/30, B21C 1/00, B21F 19/00

(54) **WIRE WITH STEEL CORE WITH A METAL ALLOY COATING**
DRAHT MIT STAHLKERN MIT EINER METALLLEGIERUNGSBESCHICHTUNG
FIL AVEC ÂME EN ACIER ET AVEC D'UN REVÊTEMENT D'ALLIAGE MÉTALLIQUE

(30) Priority: 22.06.2017 EP 17177407
(43) Date of publication of application: 29.04.2020
(73) Proprietor: NV Bekaert SA, 8550 Zwevegem (BE)
(72) Inventor: AGRESTI, Simone, 59100 Prato (IT)
(74) Representative: Messely, Marc
(86) International application number: PCT/EP2018/063955
(87) International publication number: WO 2018/233986

(56) References cited:
- JP-A- H11 179 419
- US-A- 4 686 153
- US-A1- 2003 110 612
- US-A1- 2015 360 309

## Description

### Technical Field

The invention relates to a wire having a core of steel and a metal coating and to a method of manufacturing and further processing such a wire.

### Background Art

Steel wires with a metal alloy coating, e.g. a brass coating, are known for the reinforcement of rubber products, such as rubber tires. The alloy coating is obtained by first plating the separate metals one after the other, followed by a heat treatment to diffuse the metals into an alloy. High demands are made upon these steel wires such as a high tensile strength and a high level of adhesion to rubber.

Steel wires with a metal alloy coating, e.g. a brass coating, are also known for use as loose abrasive sawing wire for the cutting of silicon ingots. As with the steel wires for rubber reinforcement, the alloy coating is here also obtained by first plating the separate metals one of the other, followed by a heat treatment to diffuse the metals into an alloy. High demands are also made upon these sawing wires such as, particularly, a high tensile strength.

It is known in the art that high tensile strengths are obtained by applying a high degree of cold deformation to the steel wires, more particularly, by means of a wet wire drawing operation with a high degree of cross-section reduction.
The state of the art of cold deformation, however, has its own inherent limits.
In order to obtain a high tensile strength, the degree of drawing has to be high. The higher the degree of drawing, the higher the losses of metal coating as a consequence of the drawing operation, more particularly as a result of the contacts between the steel wire and the drawing dies. These high losses of metal coating might be compensated by applying a thicker coating. However, this thicker coating will require a more intense heat treatment to diffuse the two metals into an alloy. The more intense this heat treatment, the higher the losses in tensile strength for the steel wire. This means that the starting tensile strength is lower, which need to be compensated by even higher degrees of drawing.
As a result, according to the state of the art and without changing other parameters such as the steel composition, there is somewhere an optimum of the obtainable final tensile strength, which is difficult to further increase without deteriorating processing.

### Disclosure of Invention

It is a primary object of the invention to further increase the obtainable tensile strength.
It is a further object of the invention to improve the deformability of steel wires.
It is also an object of the invention to reduce coating losses during deformation.
It is yet another object of the invention to reduce drawing die consumption. Viewed from another point of view, the invention also aims to reduce drawing lubricant consumption.
Still another object of the invention is to keep the adhesion in rubber products.

According to a first aspect of the present invention, there is provided a steel wire with a core of steel with a diameter ranging from 0.30 mm to 3.0 mm. The steel wire has two layers of metal coating:
1) a first layer of a zinc alloy around the steel core and clearly showing a zinc gradient with zinc being more present at the outer side;
2) a second layer of copper around this first layer.

Steel wires with a diameter ranging from 0.30 mm to 1.0 mm are suitable intermediate products to make loose abrasive sawing wire.

Steel wires with a diameter ranging from 0.90 mm to 3.0 mm are suitable intermediate products to make steel filaments adapted for rubber reinforcement.

Due to the fact that the first layer of the zinc alloy clearly shows a zinc gradient, the heating treatment for diffusion of the two or more metals in the alloy can be less intense. Hence loss of tensile strength can either be avoided or even not be present. So the intermediate steel wires have a higher starting tensile strength. As a result, for equal degrees of deformation, the final tensile strength is higher or for equal final tensile strengths, the degree of deformation can be lower.
The second top layer of copper above the first layer improves the deformability, reduces coating losses, reduces die wear and reduces lubricant consumption.

Prior art documents JP-A2-62-246425, EP-A2-0 185 492, JP-A2-61 - 284321, JP-A2-61-28432 and JP-A2-61-241027 all disclose steel wires adapted for electro-discharge machining (EDM). These steel wires have a zinc alloy coating having a zinc gradient, with zinc density becoming high towards the outer surface. Due to the fact that zinc causes a higher friction than copper and to the fact that more zinc is present at the surface, these steel wires will not have an improved drawability and neither will lead to a reduction in coating loss, a reduction in lube consumption or a reduction in die wear, on the contrary.

Prior art document WO-A1-2011/076746 discloses a brass coated steel wire with a zinc gradient in the coating. The zinc gradient is such that, in contrast to the invention, less zinc is present at the surface of the brass layer.

Prior art document EP-B1-1295 985 discloses a steel wire with two layers of metal coating. The first layer is a brass coating, the second top layer is a copper layer. EP-B1-1 295 985 does not teach the presence of a zinc gradient in the first layer. In addition, the top layer of copper has a thickness which is smaller than 0.02 µm

US4686153 is related to EDM of electrical wires and discloses creating a steel wire (11) with a copper layer (12) and with an outer CuZn-layer (14). The concentration gradient created by diffusion of the outer layer is such that concentration of zinc increases towards the outside. (See figures 2-6, abstract, columns 5-7). Hence, there is no pure upper copper layer present.

In an embodiment of the invention, the first layer is a copper-M-zinc alloy, where M is one or more metals selected from the group consisting of cobalt, nickel, tin, indium, manganese, iron, bismuth and molybdenum. The first layer and the second layer together may have a copper content ranging from 58 wt% to 75 wt%, e.g. from 61 wt% to 70 wt%. The content of the one or two metals M may range from 0.5 wt% to 10 wt%, e.g. from 2 wt% to 8 wt%.

In a preferable embodiment of the invention, the first layer is a copper-zinc alloy, only having copper and zinc as main elements.
The first layer and the second layer together may have a copper content ranging from 60 wt% to 70 wt%, e.g. from 61 wt% to 69 wt%.

The terms "clearly showing a zinc gradient with zinc being more present at the outer side" preferably refer to a configuration where there is Xout per cent of zinc at the outer side of the first layer and Xin per cent of zinc at the inner side of the first layer and where the difference Xout - Xin is more than 15 percent, e.g. more than 16 per cent, e.g. more than 17 per cent, e.g. more than 18 per cent.

In a preferable embodiment of the invention, the weight percentage of copper over the first and the second layer is more than 58 wt%.
In a preferable embodiment of the invention, the weight percentage of copper is lower than 70 wt%.

The second layer of copper has preferably a thickness more than 0.10 µm, e.g. more than 0.12 µm, e.g. more than 0.15 µm.

According to a second aspect of the invention, there is provided a method of manufacturing a steel wire. This method comprises the following steps:
a. providing a steel core with a diameter ranging between 0.30 mm and 3.0 mm;
b. plating this steel core with two or more metals, one of them being zinc;
c. heating the thus plated steel core so that the two or more metals partially diffuse and form a first layer, clearly showing a zinc gradient with zinc being more present at the outer side than the inner side;
d. plating a second layer of copper around the first layer.

Preferably, regarding the zinc gradient, there is Xout per cent of zinc at the outer side of the first layer and Xin per cent of zinc at the inner side of the first layer and where the difference Xout - Xin is more than 15 percent, e.g. more than 16 per cent, e.g. more than 17 per cent, e.g. more than 18 per cent.

In a preferable embodiment of the invention, the method further comprises the step of drawing the steel wire so that the copper of the second layer and the two or more metals of the first layer diffuse into each other and form one global layer.

Most preferably, the diffusion as a result of the drawing operation is such that the outer side of the global layer has Xgout per cent of zinc and the inner side of the global layer has Xgin per cent of zinc, where Xgout - Xgin is less than 15 per cent, e.g. less than 14 per cent, e.g. less than 12 per cent.

### Brief Description of Figures in the Drawings

Figure 1 schematically shows steps to manufacture an intermediate steel wire according to the prior art;
Figure 2 schematically shows steps to manufacture an intermediate steel wire according to the invention;
Figure 3 shows a cross-section of an intermediate steel wire according to the invention;
Figure 4 shows a cross-section of a final steel filament;

### Mode(s) for Carrying Out the Invention

Figure 1 illustrates in a schematic way a prior art process. A steel wire 10 is first plated with copper (Cu) in a copper plating installation 12 in an amount equal to the final amount of copper needed or desired. The copper plated wire is then coated with zinc (Zn) in a zinc plating installation 14 in an amount equal to the final amount of zinc needed or desired. The steel wire with the double coating is then subjected to a thermodiffusion treatment, e.g. by means of a mid-frequent installation 16. The thickness of the brass coating is represented in 17. The amount of thermodiffusion energy spent is such that a full alloying of copper with zinc is obtained, or at least approximated. This means that a gradient of zinc throughout this brass coating is non-existent or limited to maximum 15%, preferably maximum 10%. The result of this prior art process is a steel wire 18 with a more or less homogeneous brass coating.

Figure 2 illustrates the present invention. A steel wire 20 enters into a copper plating bath 22 where only 75% to 85% of the amount of finally desired or needed copper is deposited on the steel 20. Thereafter the steel wire enters into a zinc plating installation 24 where 100% of the amount of the finally desired or needed zinc is deposited. The steel wire with the double layer is then subjected to a thermodiffusion treatment in, e.g. a mid-frequent installation 26. In distinction with the prior art, only a partial alloying is aimed at, which means that only a partial diffusion is carried out thus saving 15 to 30% of thermodiffusion energy. The thickness of the partially alloyed copper-zinc coating is illustrated in 27. After the thermodiffusion step, the steel wire is plated with the remaining 25% to 15% of copper in a second copper plating installation 28.

The result is an intermediate wire 30 with a first layer of a copper-zinc alloy that is showing a clear gradient of zinc with zinc being more present at the outer side and a second layer of copper on top and around of the first layer. Due to its top copper coating, this intermediate wire 30 has a color that is more red than a wire with a common brass coating.

The partial diffusion treatment in the installation 26 bounds the zinc to copper, despite the presence of a zinc gradient. This bounding prevents the zinc from dissolving in the second copper bath 28.

Next to the degree of energy saving, the less intense thermodiffusion treatment has as additional advantage that the loss in tensile strength of the intermediate steel wire is either non-existent or substantially reduced. All other parameters being unchanged, this means that the tensile strength before the beginning of the wet wire drawing operation is higher than it is in the prior art. Tests have shown differences in tensile strength between the prior art and the invention that vary between 10 MPa and 25 MPa.

A cross-section of the double coated intermediate steel wire 30 is shown in Figure 3. The steel wire 30 has a steel core 32, a first layer of a partially alloyed copper-zinc coating 34 and a second layer of copper 36 on top of the first layer 34.

Figure 4 shows a cross-section of a final steel filament 40. It has a steel core 42 and a single 'global' layer of brass 44 without gradient or with a gradient that is less pronounced than the gradient of the intermediate steel wire 30.

As mentioned, wet wire drawing is the process that transforms the intermediate steel wire 30 into the final steel filament 40. The heat generated during the wet wire drawing process causes the first layer and the second to diffuse with each other in order to result in a brass coating that is more or less homogeneous.
In comparison with the prior art, following differences are apparent when drawing an intermediate steel wire according to the invention.
A loss of only 3% to 4% of the coating is noticed.
The wet wire drawing process consumes less lubricant.
Less energy is needed in the wet wire drawing process.
Less die wear is noticed.

These advantages can be attributed to the top copper coating 36 that causes less slip than a brass or a zinc coating.

Next to advantages experienced during wet wire drawing, the further downstream processing such as the cord twisting also has its advantages when handling a steel filament that originates from an intermediate steel wire according to the invention. More particularly, a substantial reduction in the number of fractures has been noticed. For one particular steel cord construction made by a double-twisting ("bunching") process, the level of fractures per ton was reduced with 50%.

Table 1 hereunder mentions following values and parameters:
- wire diameter of the intermediate steel wire;
- amount and thickness of the copper in the 1^{st} layer;
- amount and thickness of the zinc in the 1^{st} layer;
- amount and thickness of the copper in the 2^{nd} layer;
- Xout the percentage of zinc at the radially outer side of the 1^{st} layer after thermodiffusion;
- Xin the percentage of zinc at the radially inner side of the 1^{st} layer after thermodiffusion;
- Xout - Xin the gradient of Zn;
- the percentage of thermodiffusion energy saved in an invention process compared with the prior art.

The percentages of Zn have been measured by means of an X-ray photo electron spectroscopy (XPS) in combination with depth profiling with an argon ion gun.

**Table 1**

| Wire Diameter | 1st layer | | | | 2nd layer | | Xout | Xin | Xout - Xin | energy saved |
|---|---|---|---|---|---|---|---|---|---|---|
| | Cu | | Zn | | Cu | | | | | |
| (mm) | (g/kg) | (nm) | (g/kg) | (nm) | (g/kg) | (nm) | (%) | (%) | (%) | (%) |
| 1,65 | 2,08 | 755 | 1,51 | 688 | 0,52 | 189 | 50,3 | 27,9 | 22,4 | 20 |
| 1,09 | 3,01 | 722 | 2,09 | 629 | 0,53 | 127 | 54,1 | 17,7 | 36,4 | 17 |
| 1,85 | 1,9 | 773 | 1,36 | 694 | 0,41 | 167 | 49,7 | 26 | 23,7 | 25 |

For a final steel filament 40 the single brass coating has a zinc gradient that is much smaller than that of the first layer of an intermediate steel wire 30.

For a 0.30 mm final steel filament, a gradient Xgout - Xgin of 10% was measured, and for a 0.175 mm final steel filament, a gradient Xgout - Xgin of 11% was measured.

A suitable steel composition is e.g. a minimum carbon content of 0.65%, a manganese content ranging from 0.10% to 0.70%, a silicon content ranging from 0.05% to 0.50%, a maximum sulphur content of 0.03%, a maximum phosphorus content of 0.03%, even of 0.02%, all percentages being percentages by weight. There are only traces of copper, nickel and / or chromium. The remainder is always iron.

Micro-alloyed steel compositions may also be suitable such as compositions further comprising one or more of following elements:
- chromium (%Cr): in amounts ranging from 0.10% to 1.0%, e.g. from 0.10 to 0.50%;
- nickel (%Ni): in amounts ranging from 0.05% to 2.0%, e.g. from 0.10% to 0.60%;
- cobalt (%Co): in amounts ranging from 0.05% to 3.0%; e.g. from 0.10% to 0.60%;
- vanadium (%V): in amounts ranging from 0.05% to 1.0%, e.g. from 0.05% to 0.30%;
- molybdenum (%Mo): in amounts ranging from 0.05% to 0.60%, e.g. from 0.10% to 0.30%;
- copper (%Cu): in amounts ranging from 0.10% to 0.40%, e.g. from 0.15% to 0.30%;
- boron (%B): in amounts ranging from 0.001% to 0.010%, e.g. from 0.002% to 0.006%;
- niobium (%Nb): in amounts ranging from 0.001% to 0.50%, e.g. from 0.02% to 0.05%;
- titanium (%Ti): in amounts ranging from 0.001% to 0.50%, e.g. from 0.001% to 0.010%;
- antimony (%Sb): in amounts ranging from 0.0005% to 0.08%, e.g. from 0.0005% to 0.05%;
- calcium (%Ca): in amounts ranging from 0.001% to 0.05%, e.g. from 0.0001% to 0.01%;
- tungsten (%W): e.g. in an amount of about 0.20%;
- zirconium (%Zr): e.g. in an amount ranging from 0.01% to 0.10%;
- aluminum (%AI): preferably in amounts lower than 0.035%, e.g. lower than 0.015%, e.g. lower than 0.005%;
- nitrogen (%N): in amounts less than 0.005%;
- rare earth metals (%REM): in amounts ranging from 0.010% to 0.050%.

Within the context of the present invention low-carbon steel compositions such as disclosed in EP-A-2 268 839 are not excluded. Such a steel compositions has a carbon content of less than 0.20 %. An example is a carbon content ranging between 0.04 % and 0.08 %, a silicon content of 0.166 %, a chromium content of 0.042 %, a copper content of 0.173 %, a manganese content of 0.382 %, a molybdenum content of 0.013 %, a nitrogen content of 0.006 %, a nickel content of 0.077 %, a phosphorus content of 0.007 %, a sulphur content of 0.013 %, all percentages being percentages by weight.

### Reference numbers

- 10: steel wire
- 12: copper (Cu) plating
- 14: zinc (Zn) plating
- 16: thermodiffusion
- 17: brass coating CuZn
- 18: brass coated steel wire
- 20: steel wire
- 22: copper (Cu) plating but not to its full extent
- 24: zinc (Zn) plating
- 26: thermodiffusion but not to its full extent
- 28: top copper (Cu) plating
- 30: brass + top copper plated steel wire
- 32: steel core
- 34: first layer of brass
- 36: second layer of copper
- 40: final steel wire
- 42: steel core
- 44: layer of brass

## Claims

1. A wire
having a core of steel with a diameter ranging from 0.30 mm to 3.0 mm,
said wire having two layers of metal coating:
- a first layer of a zinc alloy around said core and clearly showing a zinc gradient with zinc being more present at the outer side,
- a second layer of copper around said first layer.

2. A wire according to claim 1,
wherein said first layer is a copper-M-zinc alloy, where M is one or two metals selected from the group consisting of cobalt, nickel, tin, indium, manganese, iron, bismuth and molybdenum.

3. A wire according to claim 1,
wherein said first layer is a copper-zinc alloy.

4. A wire according to any one of the preceding claims,
wherein said outer side of said first layer has Xout per cent of zinc and said inner side of said first layer has Xin per cent of zinc, Xout - Xin being more than 15 per cent.

5. A wire according to any one of claims 2 to 4,
wherein the weight percentage of copper over both the first and the second layer is more than 58 wt%.

6. A wire according to claim 5,
wherein the weight percentage of copper over the first and the second layer is lower than 70 wt%.

7. A wire according to any one of the preceding claims,
wherein the second layer has a thickness being more than 0.10 µm.

8. A method of manufacturing a wire, said method comprising the following steps:
a. providing a steel core with a diameter ranging between 0.30 mm and 3.0 mm;
b. plating said steel core with two or more metals, one of them being zinc;
c. heating the thus plated steel core so that the two or more metals partially diffuse and form a first layer, clearly showing a zinc gradient with zinc being more present at the outer side than the inner side;
d. plating a second layer of copper around said first layer.

9. A method according to claim 8,
wherein said outer side of said first layer has Xout per cent of zinc and said inner side of said first layer has Xin per cent of zinc, Xout - Xin being more than 15 per cent.

10. A method according to claim 8 or 9,
said method further comprising the step:
e. drawing said steel wire so that the copper of the second layer and the two or more metals of the first layer diffuse into each other and form one global layer.

11. A method according to claim 10,
wherein the diffusion as a result of said drawing is such that said outer side of said global layer has Xgout per cent of zinc and said inner side of said global layer has Xgin per cent of zinc, Xgout - Xgin being less than 15 per cent.

## Patentansprüche

1. Draht,
der einen Stahlkern mit einem 0,30 mm bis 3,0 mm betragenden Durchmesser aufweist,
wobei der Draht zwei Schichten einer Metallbeschichtung aufweist:
- eine erste Schicht einer Zinklegierung, die um den Kern verläuft und deutlich einen Zinkgradienten, bei dem mehr Zink auf der Außenseite vorliegt, aufzeigt,
- eine zweite Schicht aus Kupfer, die um die erste Schicht verläuft.

2. Draht nach Anspruch 1,
wobei es sich bei der ersten Schicht um eine Kupfer-M-Zink-Legierung handelt, wobei M für ein oder zwei aus der Gruppe bestehend aus Cobalt, Nickel, Zinn, Indium, Mangan, Eisen, Bismut und Molybdän ausgewählte Metalle steht.

3. Draht nach Anspruch 1,
wobei es sich bei der ersten Legierung um eine Kupfer-Zink-Legierung handelt.

4. Draht nach einem der vorhergehenden Ansprüche,
wobei die Außenseite der ersten Schicht Xaußen Prozent Zink und die Innenseite der ersten Schicht Xinnen Prozent Zink aufweist, wobei Xaußen - Xinnen mehr als 15 Prozent beträgt.

5. Draht nach einem der Ansprüche 2 bis 4,
wobei der Gewichtsprozentanteil an Kupfer entlang der ersten und der zweiten Schicht mehr als 58 Gew.-% beträgt.

6. Draht nach Anspruch 5,
wobei der Gewichtsprozentanteil an Kupfer entlang der ersten und der zweiten Schicht weniger als 70 Gew.-% beträgt.

7. Draht nach einem der vorhergehenden Ansprüche, wobei die zweite Schicht eine Dicke von mehr als 0,10 µm aufweist.

8. Verfahren zur Fertigung eines Drahts, wobei das Verfahren die folgenden Schritte umfasst:
a. Bereitstellen eines Stahlkerns mit einem zwischen 0,30 mm und 3,0 mm betragenden Durchmesser;
b. Abscheiden von zwei oder mehr Metallen, von denen eins Zink ist, auf den Stahlkern;
c. Erhitzen des so beschichteten Stahlkerns, sodass die zwei oder mehreren Metalle teilweise diffundieren und eine erste Schicht bilden, die deutlich einen Zinkgradienten, bei dem mehr Zink auf der Außenseite als auf der Innenseite vorliegt, aufzeigt;
d. Abscheiden einer um die erste Schicht verlaufenden zweiten Schicht aus Kupfer.

9. Verfahren nach Anspruch 8,
wobei die Außenseite der ersten Schicht Xaußen Prozent Zink und die Innenseite der ersten Schicht Xinnen Prozent Zink aufweist, wobei Xaußen - Xinnen mehr als 15 Prozent beträgt.

10. Verfahren nach Anspruch 8 oder 9,
wobei das Verfahren ferner den folgenden Schritt umfasst:
e. Ziehen des Stahldrahts, sodass das Kupfer aus der zweiten Schicht und die zwei oder mehreren Metalle aus der ersten Schicht ineinander diffundieren und eine Gesamtschicht bilden.

11. Verfahren nach Anspruch 10,
wobei Diffusion als Folge des Ziehens derart ist, dass die Außenseite der Gesamtschicht Xgaußen Prozent Zink und die Innenseite der Gesamtschicht Xginnen Prozent Zink aufweist, wobei Xgaußen - Xginnen weniger als 15 Prozent beträgt.

## Revendications

1. Fil
possédant un noyau d'acier doté d'un diamètre dans la plage de 0,30 mm à 3,0 mm, ledit fil possédant deux couches de revêtement métallique :
- une première couche d'un alliage de zinc autour dudit noyau et présentant clairement un gradient de zinc, le zinc étant plus présent au niveau du côté externe,
- une deuxième couche de cuivre autour de ladite première couche.

2. Fil selon la revendication 1,
ladite première couche étant un alliage cuivre-M-zinc, dans lequel M est un ou deux métaux choisis dans le groupe constitué par le cobalt, le nickel, l'étain, l'indium, le manganèse, le fer, le bismuth et le molybdène.

3. Fil selon la revendication 1,
ladite première couche étant un alliage cuivre-zinc.

4. Fil selon l'une quelconque des revendications précédentes,
ledit côté externe de ladite première couche possédant Xext pour cent de zinc et ledit côté interne de ladite première couche possédant Xint pour cent de zinc, Xext - Xint étant supérieur à 15 pour cent.

5. Fil selon l'une quelconque des revendications 2 à 4,
le pourcentage en poids de cuivre dans à la fois la première et la deuxième couche étant supérieur à 58 % en poids.

6. Fil selon la revendication 5,
le pourcentage en poids de cuivre dans la première et la deuxième couche étant inférieur à 70 % en poids.

7. Fil selon l'une quelconque des revendications précédentes,
la deuxième couche possédant une épaisseur supérieure à 0,10 µm.

8. Procédé de fabrication d'un fil, ledit procédé comprenant les étapes suivantes :
a. mise à disposition d'un noyau d'acier doté d'un diamètre dans la plage entre 0,30 mm et 3,0 mm ;
b. placage dudit noyau d'acier avec deux métaux ou plus, l'un d'eux étant le zinc ;
c. chauffage du noyau d'acier ainsi plaqué de sorte que les deux métaux ou plus diffusent partiellement et forment une première couche, présentant clairement un gradient de zinc, le zinc étant plus présent au niveau du côté externe que du côté interne ;
d. placage d'une deuxième couche de cuivre autour de ladite première couche.

9. Procédé selon la revendication 8,
ledit côté externe de ladite première couche possédant Xext pour cent de zinc et ledit côté interne de ladite première couche possédant Xint pour cent de zinc, Xext - Xint étant supérieur à 15 pour cent.

10. Procédé selon la revendication 8 ou 9,
ledit procédé comprenant en outre l'étape de :
e. tirage dudit fil d'acier de sorte que le cuivre de la deuxième couche et les deux métaux ou plus de la première couche diffusent l'un dans l'autre et forment une couche globale.

11. Procédé selon la revendication 10,
la diffusion résultant dudit tirage étant telle que ledit côté externe de ladite couche globale possède Xgext pour cent de zinc et ledit côté interne de ladite couche globale possède Xgint pour cent de zinc, Xgext - Xgint étant inférieur à 15 pour cent.
